

# United States Patent

Cassella, Jr.

[15] 3,668,124

[45] June 6, 1972

[54] **COMPOSITION AND METHOD FOR  
TREATING DRY-CLEANABLE SOIL-  
RESISTANT LEATHERS**

[72] Inventor: **Vincent Joseph Cassella, Jr.**, Audubon, Pa.  
[73] Assignee: **Pennwalt Corporation**, Philadelphia, Pa.  
[22] Filed: **May 13, 1970**  
[21] Appl. No.: **37,019**

[52] U.S. Cl. .... **252/8.57**, 8/94.22, 8/94.23  
[51] Int. Cl. .... **C14c 5/00**, C14c 9/00  
[58] Field of Search ..... 8/94.22; 252/8.57

[56] **References Cited**

UNITED STATES PATENTS

2,974,000 3/1961 Retzsch ..... 8/94.23

OTHER PUBLICATIONS

W. J. Hopkins et al. JALCA 62, pages 162-163 (1967).

Primary Examiner—George F. Lesmes  
Assistant Examiner—M. B. Wittenberg  
Attorney—Stanley Litz and Carl A. Hechmer, Jr.

[57] **ABSTRACT**

A fat liquor composition useful for leather treatment comprises a mixture of alkenyl substituted succinic acid or succinic acid anhydride, sulfated fatty oil, and an amine or amide. The leather is treated with an aqueous emulsion of the fat liquor composition and then with an aqueous solution of the chromium coordination complex of perfluoroalkyl-containing carboxylic acid to provide a soil and water-repellent leather that is resistant to loss of lubricity when dry cleaned.

5 Claims, No Drawings

## COMPOSITION AND METHOD FOR TREATING DRY-CLEANABLE SOIL-RESISTANT LEATHERS

This invention relates to a composition and method for lubricating and imparting softness, and soil and water repellency to leather. More particularly, this invention concerns treating leather with a fat-liquoring composition comprised of a mixture of alkenyl succinic acid or acid anhydride, a sulfated fatty oil, and an organic, nitrogen-containing compound, such as an amine or amide, followed by treatment with a chromium coordination complex of a perfluoroalkyl-containing carboxylic acid.

There are several significant and important advantages achieved by the use of the composition and the practice of the method of the present invention. Leather treated according to this invention, especially suede garment leathers made of sheepskin or cow-hide split, can be drycleaned in conventional drycleaning equipment without loss of softness caused by extraction of the lubricating oils from the leather by the cleaning solvent. In addition to its resistance to extractability of lubricating (fat liquor) oils, leather treated according to this invention is notably resistant to water and oil-borne stains. Moreover, when staining does occur, the stain can be easily removed by a damp cloth or with aerosol spot removers. Leather garments made from leathers treated in accordance with the invention are especially attractive to consumers since problems long associated with such clothing are alleviated, for example, water spotting after wetting and the difficulty of removing stains, soils and dirt from the leather.

Moreover, an important advantage of this invention accruing to the tanner or manufacturer is that much less fat liquor composition is required to lubricate the leather compared to that required with the conventional fat liquors used prior hereto. For example, 0.5 to 1.5 percent by weight of the fat liquor lubricating composition of this invention, based on the weight of leather, will lubricate sheep skin garment suede to give a satisfactory soft hand and drape compared to 8 to 12 percent of conventional oils required in the present practice in the industry. Similarly, the amount of the fat liquor composition of this invention required to satisfactorily lubricate split garment leather is 4 to 6 percent of the leather weight compared to 18 to 26 percent required for conventional oils.

The fat liquor lubricating composition used in the first step of the leather treatment process of this invention comprises a mixture of from about 30 to about 90 parts by weight of alkenyl substituted succinic acid or alkenyl substituted succinic acid anhydride wherein the alkenyl group attached to the alpha carbon atom of the acid or anhydride has from about 12 to 24 (preferably 15 to 20) carbon atoms; from about five to about 60 parts (preferably 10 to 40) parts by weight of sulfated fatty oil, and about five to 25 (preferably about 10 to 15) parts by weight of an organic, nitrogen-containing compound selected from the group consisting of alkyl amines, alkanol amines, heterocyclic amines, aromatic amines, and alkyl amides. The alkenyl succinic acid or anhydride may of course be a mixture of acids or anhydrides having alkenyl groups of varying chain lengths within the aforesaid range.

The standard term "sulfated fatty oil" refers to those conventional fat-liquoring oils containing at least 4 percent by weight of combined sulfate (SO<sub>4</sub><sup>2-</sup>). Examples of such known, highly sulfated fat-liquoring oils are the sulfated vegetable, fish, and animal fat oils such as sulfated olive oil, mahogany oil, cotton seed oil, corn oil, peanut oil, soy beam oil, palm oil, cod oil, neatsfoot oil, sperm oil and others known in the art. It has been found that the pure unsulfated fatty oils, as well as mineral oil, when substituted for the sulfated oil of the claimed composition, do not provide the desired results.

The organic, nitrogen-containing compound in the fat-liquoring composition of this invention is necessary to aid in emulsification of the fat-liquoring composition in the aqueous media which is normally used in leather treatment. Representative of such nitrogen containing compounds are alkyl amines, alkanol amines, aromatic amines, heterocyclic amines and alkyl amides, e.g., the mono-, bi-, and tri-alkyl amines, the methyl amines, hexyl amines octyl amines, decyl amines, i.e.,

wherein the alkyl group has up to about 12 carbon atoms; the hydroxyl-containing alkyl amines such as the mono-, bi- and tri-ethanol amines and propanol amines, methyl diethanol amine, 2-aminopropanol, dimethylamino ethanol, diglycol amine, and the like; heterocyclic amines such as morpholine and piperidine and the like; aromatic amines, such as analine, toluidine, n-methylaniline and the like; and representative amides such as dimethylformamide, dimethylacetamide, diethylacetamide, dimethylpropionamide and the like.

- 10 The fatliquor composition of this invention as above described is a slightly viscous to very viscous oil in physical appearance. Preparatory to treatment of leather with this fatliquor composition, it is advantageously mixed with from 15 about 300 to 700 parts by weight of water per hundred parts by weight of the fatliquor composition, preferably at a temperature within the range of about 115° F. to about 130° F., with vigorous stirring, to provide an oil-in-water emulsion medium which is subsequently applied to the leather by conventional drumming techniques well known to those skilled in the art of leather treatment. For example, the leather is treated with the fatliquor composition by contact therewith for from about 30 to 60 minutes at somewhat elevated temperatures, preferably ranging from about 115° F. to about 20 130° F. It is generally advantageous to first drum the washed skins in hot water to ensure they are thoroughly wetted prior to fatliquoring.

25 The second step of the process of this invention involves contacting the leather, which has previously been treated with 30 the aforesaid lubricant composition, with a chromium coordination complex of a perfluoroalkyl carboxylic acid, wherein the perfluoroalkyl group (linear or branched chain) embodied therein desirably contains from about six to about 18 carbon atoms, preferably nine to 15 carbon atoms. Representative 35 complexes are described in U.S. Pat. No. 3,351,643 which discloses chromium coordination complexes of perfluoroalkyl acids of the structure



40 where R<sub>1</sub> is perfluoroalkyl, R is hydrogen or alkyl having one to four carbon atoms and R' is alkylene having one to six carbon atoms; and U.S. Pat. No. 2,934,450 which describes 45 chromium coordination complexes of perfluoroalkyl acids having the structure



50 where R<sub>1</sub> is the perfluoroalkyl group, R is hydrogen or alkyl having one to six carbon atoms and R' is an alkylene group having from one to 12 carbon atoms. Other perfluoroalkyl 55 carboxylic acids of this type which may be converted into chromium coordination complexes essentially in the manner described in the foregoing patents and used in the second step of the process of this invention are represented by the following (where n and m integers as described in the references):



- 60 65 and the other fluoroalkyl acids described in U.S. Pat. No. 3,471,518; R<sub>1</sub>COOH as described in U.S. Pat. No. 3,311,566; R<sub>1</sub>(CH<sub>2</sub>)COOH as described in U.S. Pat. No. 2,951,051; R<sub>1</sub>(CH<sub>2</sub>)<sub>n</sub>S(CH<sub>2</sub>)<sub>m</sub>COOH as described in U.S. Pat. No. 3,172,910; R<sub>1</sub>O(CF<sub>2</sub>)<sub>n</sub>COOH and R<sub>1</sub>O(CF<sub>2</sub>)<sub>n</sub>(CH<sub>2</sub>)<sub>m</sub>COOH as 70 described in U.S. Pat. No. 3,453,333; R<sub>1</sub>O(CF(CF<sub>3</sub>)CF<sub>2</sub>O)<sub>n</sub>CF(CF<sub>3</sub>)COOH as described in U.S. Pat. No. 3,274,239 and U.S. Pat. No. 3,250,808; R<sub>1</sub>(CH<sub>2</sub>)<sub>n</sub>O(CH<sub>2</sub>)<sub>m</sub>COOH and other acids described in U.S. Pat. Nos. 3,231,604 and 3,145,222; and R<sub>1</sub>CH(OH)COOH described in U.S. Pat. No. 3,202,706, and other like fluoroalkyl acids.

The chromium coordination complexes of perfluoroalkyl carboxylic acids are conveniently water-soluble, and, therefore, dilute aqueous solutions thereof are advantageously used to treat the leather subsequent to the fatliquor treatment step described previously. For example, aqueous solutions containing from about 0.5 percent to 7 percent by weight of the chromium coordination complex are preferably used to give a pick-up of the chrome complex on the leather of approximately the same concentration based on the blue weight of the leather. The pH of the chromium complex treating solution will range from about 3 to 5.5, preferably from 3 to 3.5, and this pH is adjusted, if necessary, by the addition thereto of a small amount of an organic acid or mineral acid such as formic acid, acetic acid or sulfuric acid. The leather is treated with the chromium coordination complex solution at a temperature in the range of about 100° to 130° F. for from about 15 to 60 minutes.

After drying, and, if desired, staking and buffing, the treated skins show unusually good repellency to water and oil spotting and resistance to oil- and water-borne stains, in addition to being comparatively quite resistant to oil extraction in dry cleaning. The skins also show a pronounced improvement in softness, in hand and in drape, making highly desirable for suede garment manufacture.

The following examples are presented to illustrate the invention and to demonstrate that all elements described therein are necessary in order to give the stated results. Unless otherwise stated, all amounts of ingredients referred to in the examples are given in parts by weight.

#### EXAMPLE 1

A fat liquor composition in accordance with this invention is prepared by blending 10 parts of morpholine with 80 parts of mixed alkenyl succinic acid anhydride wherein the alkenyl substituent ranges from C<sub>15</sub> to C<sub>20</sub> ("Chevron ASA," a product of Chevron Chemical Company), and this is mixed with 10 parts of sulfated sperm oil ("Hydrol 80," product of Reilly-Whiteman-Walton Company.)

Tanned sheepskins taken from production following extract retanning are washed, short floated at 120° F., and drummed for 20 minutes. The emulsified fatliquor composition is added to the leather treatment wheel (1 percent based on the wet weight of the skins). The skins are drummed for 40 minutes at 120° F., and the float appears clear. The skins are then rinsed for 5 minutes at 110° F., horsed overnight (14-16 hours), and then set out (put through a wringer to remove excess water), tunnel dried overnight, milled, and buffed.

The fat liquor treated skins are wet back for 30 minutes at 130° F. and again medium to short floated at 120° F. The float is adjusted to pH 3 to 3.5 with formic acid. Then 2.5 percent (based on weight of the blue skins) of a chromium coordination complex of a branched perfluoroalkyl acid (having the formula



where R<sub>1</sub> (i.e., (CF<sub>3</sub>)<sub>2</sub>CF(CF<sub>3</sub>)<sub>n</sub>) is a mixture of from nine to 15 fluoroalkyl carbon atoms, U.S. Pat. No. 3,351,643) is added to an equal amount of hot water (120° F.) and the mixture added to the drum. The skins are drummed 45 minutes after which time the bath is clear. The skins are rinsed at 100° F. for 5 minutes and then horsed. After a minimum of 2-3 hours, the skins are toggle dried and put through the final stages of staking and blocking.

The treated leather has excellent water and oil repellency properties. The leather is passed through a typical coin-operated dry-cleaning cycle and the results show there is a 9.1 percent loss of fat liquor lubricant in the drycleaning operation.

#### EXAMPLE 2

The procedure of Example 1 is repeated, except that the fat liquor composition added to the leather is 1 percent of the alkenyl substituted succinic acid anhydride ("Chevron ASA") without the addition of sulfated fatty oil and amine. The lubrication step is followed by treatment with 2 percent of the chromium coordination complex of the perfluoroalkyl-containing carboxylic acid as in Example 1. The loss in drycleaning of the fat liquor lubricant is significantly greater (23.8 percent) for this leather.

#### EXAMPLE 3

The procedure of Example 2 is repeated, except that the amount of alkenyl substituted succinic acid anhydride added to the leather is increased to 3 percent. This reduces the fat loss in dry cleaning to 8 percent. However, the treating materials do not penetrate the leather sufficiently and there is an unacceptable greasy deposit on the surface of the skin.

#### EXAMPLE 4

The fat-liquoring treatment of Example 1 is repeated, using 8 percent by weight of fatty oils of the mayonnaise type ("Nutreene ED and Nutreene X," products of Salem Oil and Grease Company). The treatment of the leather with the chromium coordination complex of the perfluoroalkyl-containing carboxylic acid is omitted. The fat loss after one drycleaning cycle is 65 percent of the lubricant originally applied.

#### EXAMPLE 5

Fifty parts of "Chevron ASA" are blended with 10 parts of morpholine and 40 parts of a sulfated mixture of fatty oils and alcohol fatty esters (Reilly-Whiteman-Walton "938X fat liquor"). The fat liquor composition is emulsified with water (120° F.), added to the wheel, and used to treat 100 pounds of split garment leather which had first been washed, short floated at 120° F. and drummed for 20 minutes. Ten percent of the fat liquor lubricant composition based on wet weight is taken up by the leather. The skins are drummed for 45 minutes, rinsed for 5 minutes at 110° F. and refloated (short) at 120° F. The float is adjusted to pH 3 to 3.5 with formic acid, and 2.5 percent of the chromium coordination complex used in Example 1 (based on blue weight of the skins) is added to an equal amount of hot water (120° F.), and the solution added to the wheel. The skins are drummed 45 minutes, after which the float is clear. The skins are water-rinsed for 5 minutes at 110° F., dumped, horsed overnight, hung dried at 100° F. for 5 hours, and then put through the final stages of staking and buffing. The skins show very good water and oil repellency as well as resistance to water- and oil-borne stains.

The skins are subjected to a coin operated drycleaning cycle operation and only 6.6 percent of the fat liquor lubricant is lost in the drycleaning.

I claim:

1. A fat liquor lubricating composition useful for the treatment of leather comprising a mixture of from about 30 to about 90 parts by weight of alkenyl substituted succinic acid or alkenyl substituted succinic acid anhydride wherein the alkenyl group attached to the alpha carbon atom of the acid or anhydride contains from about 12 to 24 carbon atoms, from about five to about 60 parts by weight of sulfated fatty oil, and about five to 25 parts by weight of an organic, nitrogen-containing compound selected from the group consisting of alkyl amines, alkanol amines, heterocyclic amines, aromatic amines, and alkyl amides.
2. The composition in accordance with claim 1 wherein the alkenyl group of the substituted succinic acid or anhydride has from 15 to 20 carbon atoms.
3. The composition in accordance with claim 1 wherein the organic, nitrogen-containing compound is morpholine.

4. The composition in accordance with claim 1 wherein there are from 10 to 40 parts by weight of sulfated fatty oil and about 10 to 15 parts by weight of the nitrogen-containing compound.

5. The composition in accordance with claim 4 wherein the alkenyl group of the substituted succinic acid or anhydride has from 15 to 20 carbon atoms.

\* \* \* \* \*

10

15

20

25

30

35

40

45

50

55

60

65

70

75